

## UNITED STATES PATENT OFFICE.

GEORGE W. CHILDS, OF NEW YORK, N. Y.

## LIQUID LEATHER-DRESSING.

No. 875,653.

Specification of Letters Patent.

Patented Dec. 31, 1907.

Original application filed May 16, 1906, Serial No. 317,141. Divided and this application filed August 30, 1907. Serial No. 390,763.

*To all whom it may concern:*

Be it known that I, GEORGE W. CHILDS, of New York city, in the county and State of New York, have invented a certain new and useful Improvement in Liquid Leather-Dressings, whereof the following is a specification.

This application is a division of my application Serial #317,141 filed May 16, 1906, and 10 the claims herein are limited to a dressing adapted for impregnating leather to increase the ultimate solidity of the latter when dried, and containing solid matter derived from sapped or exhausted organic tanning liquors. 15 As described in my original application aforesaid, such sapped liquors being usually polluted with chemicals introduced thereto or resulting from chemical changes therein, and carrying a large percentage of non-tannic material, are termed "runaway" or "taii" 20 liquors and are ordinarily discharged to waste from the last layer in which they have been sapped.

To produce the dressing herein claimed, I 25 treat the spent liquor in accordance with the nature of the same, as follows:—If the spent liquor contains lime or lime compounds, these components may be precipitated by the addition of chemicals forming insoluble 30 compounds with lime. For instance, ammonium oxalate, sodium phosphate, sodium fluorid or carbon dioxide gas may be employed to effect such precipitation. The precipitate is then settled out and the super- 35 natant liquor run off for further purification or concentration. If the spent liquor contains non-volatile impurities, such as mineral acids, these may be either neutralized by the addition of alkali, such as sodium hydrate or 40 potassium hydrate or may be precipitated by the addition of bases forming insoluble compounds with the acids, such as barium chlorid. Said spent liquor may then be heated until the volatile impurities, for instance, acetic or pro- 45 pionic or butyric acids, are eliminated and the resultant liquid is concentrated, conveniently by continued heating *in vacuo*, until it at- tains a specific gravity of 1.05 to 1.3.

The otherwise waste liquors thus purified 50 and concentrated may be utilized to increase the solidity of leather as follows:—Hides

which have been subjected to the action of a tanning solution until they have combined with approximately all the tannin with which they will combine, are then impregnated with 55 the concentrated waste tanning liquor, in any convenient manner, for instance, such leather may be placed in a rotary drum and said concentrate, preferably heated, introduced to said drum, conveniently through a hollow 60 axle or trunnion thereof, and the revolution of said drum continued until said concentrate is absorbed by the leather and fills the pores of the latter so that when dried the residue of the liquor in the leather, not only renders 65 the latter more solid than if it had not been impregnated with said liquor, but also adds materially to its final weight. It may be observed that if said liquors are not concentrated to substantially the consistency 70 described, there will not be sufficient solid residue thereof when the leather is dried, to attain the result desired. Moreover, if the liquors are concentrated to a greater degree they will not be absorbed by the leather. 75 Leather impregnated as last described may then be bleached, oiled, dried, dampened, and rolled in the usual manner.

I do not desire to limit myself to all the details of procedure above enumerated, as 80 various modifications may be made therein without departing from the essential features of my invention as defined in the appended claims.

I claim:—

1. A leather dressing adapted for impregnating leather, derived from sapped or exhausted organic tanning liquor and having a specific gravity of from 1.05 to 1.3, substantially as described. 85

2. A leather dressing adapted for impregnating leather, containing inert solid matter derived from sapped or exhausted organic tanning liquors and having a specific gravity of from 1.05 to 1.3, substantially as described. 90

In testimony whereof, I have hereunto signed my name at New York, New York, this 26th day of August, 1907.

GEORGE W. CHILDS.

Witnesses:

W. G. HORTON,  
F. P. PALM.